

Sept. 3, 1957

P. N. RYLANDER ET AL. 2,805,187  
METHOD OF DESULFURIZING HYDROCARBON OIL USING HYDROGEN  
AND A COBALT FERRITE OR NICKEL FERRITE CATALYST  
Filed April 30, 1956



INVENTORS:

Paul N. Rylander  
Wilford J. Zimmerschied

BY Joseph C. Kotarski

ATTORNEY

1

2,805,187

## METHOD OF DESULFURIZING HYDROCARBON OIL USING HYDROGEN AND A COBALT FERRITE OR NICKEL FERRITE CATALYST

Paul N. Rylander, Chicago, Ill., and Wilford J. Zimmerman, Crown Point, Ind., assignors to Standard Oil Company, Chicago, Ill., a corporation of Indiana

Application April 30, 1956, Serial No. 581,498

8 Claims. (Cl. 196—28)

This invention relates to the desulfurizing of hydrocarbon oils and in particular it concerns the use of novel catalysts for the hydrodesulfurization of hydrocarbon oils containing organic sulfur compounds. This application is a continuation-in-part of our Serial No. 535,269, filed September 19, 1955 and now abandoned.

Petroleum or other hydrocarbon oils which contain appreciable amounts of sulfur compounds are objectionable for use as fuel, lubricating oils, solvents, or cracking stocks and the like. Frequently virgin and cracked naphthas must be desulfurized before blending into gasoline or before further processing, such as hydroforming, to improve their octane number. The high sulfur components, e. g. coke still naphtha, of gasoline require desulfurization in order to produce a blended gasoline meeting the requirement of low sulfur content. A number of catalysts are available for the hydrodesulfurization of virgin naphthas, but if they are employed in hydrodesulfurizing olefinic naphthas such as thermally or catalytically cracked naphthas, they catalyze indiscriminate desulfurization and hydrogenation of the higher octane olefins to produce lower octane paraffins. The olefinic naphthas, e. g. coke still naphtha, may suffer a loss of 10 to 20 octane numbers. In addition, a considerable amount of expensive hydrogen is used in saturating the olefins.

An object of this invention is to provide a method and means for desulfurizing hydrocarbon oils which utilizes highly active and effective hydrodesulfurization catalysts. Another object is to provide selective desulfurization catalysts useful for desulfurizing olefinic hydrocarbon oils with a minimum consumption of hydrogen. An important object of this invention is to provide an economical method and means for achieving a high degree of desulfurization of olefinic naphthas while maintaining saturation, i. e. hydrogenation, of the olefinic components at a minimum and thereby obtaining a desulfurized olefinic naphtha whose octane number has not been substantially reduced during hydrodesulfurization. Other objects will become apparent from the detailed description of our invention.

It has been discovered that cobaltous ferrite and nickelous ferrite, which are chemical compounds having a spinel structure and corresponding with the formulae  $\text{CoFe}_2\text{O}_4$  and  $\text{NiFe}_2\text{O}_4$  respectively, are highly effective catalysts for the hydrodesulfurization of hydrocarbon oils. They may be employed alone or as the essential components of a contact or catalyst mass. Desulfurization of the hydrocarbon oil may be carried out by contacting the oil at a temperature between about 600° and 1000° F. in the presence of hydrogen, usually under a hydrogen partial pressure of between 100 and 3000 p. s. i. g. (but preferably less than 1500 p. s. i. g.  $\text{H}_2$  if an olefinic naphtha is used) with the cobaltous ferrite or nickelous ferrite catalyst. A high degree of desulfurization of the olefinic naphtha is obtained along with a much lesser degree of hydrogenation of the olefinic constituents of the naphtha.

Cobaltous ferrite and nickelous ferrite are not mere

2

physical mixtures of their metal oxide components (cobalt oxide plus ferric oxide and nickel oxide plus ferric oxide, respectively). They are true chemical compounds which have a spinel type structure. In the spinel structure the oxygen atoms are arranged on a face-centered cubic lattice, in cubic close packing, the cobalt or nickel atoms being surrounded by tetrahedral groups of four oxygen atoms and the ferric atoms by octahedral groups of six atoms. These metal ferrites are para-magnetic.

10 Cobaltous ferrite has a cubic structure which measures 8.36° A along the side and has a molecular volume of  $584 \times 10^{-24}$  cc. It is brown in color and has a specific gravity of 5.19. Nickelous ferrite measures 8.43° A along the side and has a molecular volume of  $580.09 \times 10^{-24}$  cc. It is brown in color and has a specific gravity of 5.268.

The metal ferrite may be prepared by commingling a cobalt and/or nickel compound which affords the oxide of cobalt and/or nickel with an iron compound which affords an oxide of iron, and then calcining the intimate mixture by heating it at a temperature between about 1400° and 2000° F. for a period of about 1 to 24 hours. Cobalt compounds which may be used are inorganic cobalt compounds such as  $\text{CoCO}_3$ ,  $2\text{CoCO}_3 \cdot 3\text{Co(OH)}_2 \cdot \text{H}_2\text{O}$ ,  $\text{Co(OH)}_2$ ,  $\text{Co}_2\text{O}_3 \cdot 3\text{H}_2\text{O}$ ,  $\text{CoO}$ ,  $\text{Co}_3\text{O}_4$ ,  $\text{Co}_2\text{O}_3$ ,

$$\text{Co}(\text{NO}_3)_2 \cdot 6\text{H}_2\text{O}$$

as well as organic cobalt compounds such as  $\text{CoC}_2\text{O}_4$  and the like. When preparing the nickelous ferrite catalyst, 30 compounds which afford nickel oxide at the elevated calcination temperature, and which are therefore useful in preparing the nickelous ferrite catalyst, are those such as  $\text{NiO}$ ;  $\text{Ni}_2\text{O}_3$ ;  $\text{Ni}_3\text{O}_4$ ;  $\text{Ni}_3\text{O}_4 \cdot 2\text{H}_2\text{O}$ ;  $\text{Ni}(\text{OH})_3$ ;

35  $\text{Ni}(\text{OH})_2 \cdot \frac{1}{2}\text{H}_2\text{O}$ ;  $\text{NiCO}_3$ ;  $2\text{NiCO}_3 \cdot 3\text{Ni}(\text{OH})_2 \cdot 4\text{H}_2\text{O}$ ;  $\text{NiCl}_2 \cdot 6\text{H}_2\text{O}$ ;  $\text{Ni}(\text{HCO}_3)_2 \cdot 2\text{H}_2\text{O}$  (nickel formate);  $\text{Ni}(\text{C}_2\text{H}_3\text{O}_2)_2$  (nickel acetate). The iron compounds employed in forming the cobaltous or nickelous ferrite are usually inorganic ferric and ferrous compounds such as  $\text{Fe}(\text{OH})_3$ ,  $\text{Fe}(\text{OH})_2$ ,  $\text{Fe}_2\text{O}_3$ ,  $\text{FeO}$ ,  $\text{Fe}_3\text{O}_4$ ,  $\text{FeF}_2$ ,  $\text{FeCl}_2$ ,  $\text{FeCl}_3$ ,  $\text{Fe}(\text{NO}_3)_3 \cdot 6$  or  $9\text{H}_2\text{O}$ ,  $\text{Fe}(\text{NO}_3)_2 \cdot 6\text{H}_2\text{O}$ , as well as organic iron compounds such as

$$\text{Fe}(\text{C}_3\text{H}_5\text{O}_3)_2 \cdot 3\text{H}_2\text{O}$$

40 45 (ferrous lactate),  $\text{Fe}_2(\text{C}_2\text{O}_4)_3$  (ferric oxalate),  $\text{Fe}(\text{CHO}_2)_3$

(ferric formate) and the like. When preparing the cobaltous ferric catalyst a mixture of  $\text{CoNO}_3 \cdot 6\text{H}_2\text{O}$  and  $\text{FeNO}_3 \cdot 9\text{H}_2\text{O}$  may conveniently be employed because as the two materials are heated a liquid is formed which mixes thoroughly as water is boiled off and the temperature raised to the level necessary to form the cobaltous ferrite. A mixture of nickel oxide and ferric oxide are highly suitable for use in preparing the nickelous ferrite catalyst.

50 55 The cobalt and/or nickel compounds and the iron compound are intimately mixed in the desired proportions before being calcined. The intimate mixture of the cobalt and/or nickel compound with the iron compound should contain the cobalt and/or nickel and the iron in a molar ratio of approximately 0.2 to 2.0 mols of cobalt and/or nickel per mol of iron. Since the molar ratio of cobalt to iron and the molar ratio of nickel to iron in the cobaltous ferrite and nickelous ferrites respectively, is 1:2, the use of an excess of either the iron or the cobalt and/or nickel in the mixture which is heated serves no especially useful function but serves merely as an extender for the cobaltous ferrite or the nickelous ferrite. Thus it is preferred to calcine a mixture which contains a cobalt to iron molar ratio of 1:2 or a nickel to iron molar ratio of 1:2.

The cobalt and/or nickel compound is intimately mixed with the iron compound before calcination. This may be done by ball milling the particular cobalt and/or nickel compound with the iron compound in the dry or wet state, preferably the latter. For example, a water or methanol slurry of the mixture may be ball milled until finely ground and mixed. If the cobalt and/or nickel together with the iron compounds are completely soluble in a minor amount of water, vigorous mixing is not necessary. After an intimate mixture is obtained, the water, methanol, or whatever slurring medium is used, is vaporized in a separate step or during the early stages of the calcination. While this intimate mixture may be calcined at a temperature between about 1400° and 2000° F. or higher, a temperature of at least about 1800° F. is preferred. It is essential to carry out the calcination at a temperature of at least 1400° F. in order to obtain an active catalyst; for if the calcination is carried out at a much lower temperature e. g. 1200° F. or less, or if the mixture of the cobalt and/or nickel compound with the iron compound is not calcined (heated) at all, the product will have only weak and unsatisfactory ability to catalyze hydrodesulfurization. The calcination may be carried out over a course of 1 to 24 hours or more, suitably 3 to 18 hours. Because the catalytic material is produced at such an elevated temperature and is stable at such temperatures, it has an inherent advantage over other desulfurization catalysts wherein the temperature of regeneration of the catalyst must be carefully controlled to about 1200° F. or lower to avoid sintering and deactivation.

The calcination product may be used in a desulfurization process in the form of fragments as obtained from the calcination step, or it may be pulverized and pelleted with the aid of 1-2% of Sterotex (hydrogenated corn oil), stearic acid, or the like which are employed as binders and subsequently burned from the pellets. If the catalyst is employed in pelleted form, it can be pelleted together with a carrier such as activated alumina, bauxite, or the like. The various carriers or spacing agents, upon which the calcination product may be extended, can be incorporated in the finished catalyst by pulverizing the carrier material e. g. activated alumina, hydrous alumina gel, commingling it with the pulverized calcination product, then pelleting it with the aid of a binder, and finally burning the binder therefrom with dilute oxygen at a temperature of about 500 to 1000° F. (but not higher than 1200° F.). While the cobaltous ferrite or the nickelous ferrite may be extended upon a carrier material to reduced the cost, it is preferred to use an unsupported metal ferrite catalyst when desulfurizing an olefinic naphtha because the unsupported catalyst generally displays a greater preference for desulfurization rather than paraffination of the olefins (which are generally of higher octane number than the corresponding paraffins).

Hydrocarbon oils which may be desulfurized are those such as petroleum and fractions thereof, coal hydrogenation oils, shale oil, and the like which contain objectionable amounts of sulfur compounds, nitrogen compounds and oxygen compounds. The oil may be a virgin or cracked distillate. Virgin or cracked naphthas are particularly suitable feeds to the process of this invention, although higher boiling oils e. g. kerosene, gas oil, etc. may be employed. Olefinic naphthas such as contain an olefin to paraffin ratio in the range of 3:1 to 1:3 are particularly suitable feed stocks because minimum saturation of the olefin content occurs during the hydrodesulfurization process. An outstanding example of a high sulfur olefinic naphtha is a naphtha produced by the coking of a high sulfur reduced crude by conventional methods such as delayed coking or fluidized coking methods. Such a naphtha is exceedingly more difficult to desulfurize by conventional methods than are the olefinic naphthas produced by thermal cracking or by catalytic cracking.

The hydrocarbon oil is desulfurized by passing it

together with hydrogen through the reactor containing the catalyst. The catalyst may be contained in the reactor in tubes, trays, or other appropriate containers, or it may be employed in the fluidized state. The conditions employed in desulfurization when using our catalyst will of course vary to some extent dependent upon the type of hydrocarbon oil to be desulfurized and the extent of desulfurization desired. A temperature of 600 to 1000° F. may be used, the higher temperatures being employed in desulfurizing higher boiling feed stocks. When desulfurizing naphtha fractions a temperature of about 600 to 800° F., preferably about 750° F., may be employed. Under such conditions the naphtha is desulfurized while in the vapor state, whereas when desulfurizing a gas oil, a liquid phase is present. A pressure ranging from about 100 or 3000 p. s. i. g. or higher may be employed in the reactor. The oil is contacted with the catalyst in the presence of hydrogen which may be employed in the amount of 500 to 5000, preferably 1500 to 3000 s. c. f./bbl. oil. The hydrogen may consist of introduced outside hydrogen as is employed in a conventional hydrofining type operation, or it may be generated within the reactor by dehydrogenation of the naphthenes present in the feed stock as occurs in "autofining." Space velocities of between 0.5 to as high as 20 volumes of oil per hour per volume of catalyst, preferably between 2 to 10 volumes of oil per hour per volume of catalyst, may be employed.

The higher space velocities are used with the more easily desulfurized stocks such as virgin naphtha, whereas the lower space velocities of about 2 to 5 are employed with the more difficultly desulfurized stocks such as coke still naphtha, higher boiling stocks such as gas oils, and the like.

After the catalyst has been used for a sufficient length of time so that its activity begins to decline, it may be regenerated by burning the hydrocarbonaceous material therefrom employing diluted oxygen such as a mixture of flue gas with air. Because of the thermal stability of the catalyst, the temperature of regeneration need not be kept below 1200° F. as is necessary to avoid deactivation of presently available commercial hydrodesulfurization catalysts. The temperature may be as high as about 1600°-1800° F. Regeneration at these higher temperatures is more rapid and the down-time of the hydrodesulfurization unit can be decreased. Not only will the use of our catalyst minimize costly equipment necessary to control regeneration of the catalyst, but it will have the added economic incentive of reducing unit down-time.

The effectiveness of the nickelous ferrite as a catalyst for hydrodesulfurizing hydrocarbon oils was demonstrated in a number of experiments. These experiments show the extreme importance of carrying out the calcination of the nickel compound and the iron compound at a temperature of 1400° F. or higher in order to obtain nickelous ferrite which is highly active as a desulfurization catalyst. Five different catalytic materials were prepared and their effectiveness evaluated for desulfurizing a coke still naphtha. The catalysts used in runs 1 through 3 inclusive were prepared by calcining (using different calcination temperatures in preparing each catalyst) an intimate mixture of one mol of NiO and one mol of Fe<sub>2</sub>O<sub>3</sub> (the mixture thus having a molar ratio of nickel to iron of 0.5:1). The catalyst used in runs 4 and 5 was prepared from an intimate mixture of NiCO<sub>3</sub> and Fe<sub>2</sub>O<sub>3</sub>. The catalyst used in run 4 was prepared by calcining a mixture containing one mol of NiCO<sub>3</sub> and one mol of Fe<sub>2</sub>O<sub>3</sub> (0.5 mol of nickel per mol of iron), and the catalyst used in run 5 was prepared from a mixture containing 2 mols of NiCO<sub>3</sub> and 1 mol of Fe<sub>2</sub>O<sub>3</sub> (1.0 mol of nickel per mol of iron). The technique employed in preparing the catalysts was to ball mill a mixture of the nickel compound and the iron compound with methanol, dry the resultant slurry, and then calcine it for about 18 to 24

hours at the defined calcination temperature. The fragments produced upon calcination of the mixtures was ground and then employed in the hydrodesulfurization runs.

In carrying out the hydrodesulfurization runs, samples of the catalyst compositions to be tested were placed in the center section of an electrically heated one-inch (id.) stainless steel vertical reactor approximately 38 inches long. The section above the catalyst was packed with glass beads to act as a preheat section for the incoming feed. Samples of coke still naphtha (which were obtained from the delayed coking of a mixture of high sulfur reduced crudes primarily of West Texas origin) having sulfur contents ranging between 0.55 and 0.65 and bromine numbers of approximately 70 were passed together with once-through hydrogen (at a rate approximating 2000 standard cubic feet of hydrogen per bbl. of naphtha) through the top of the downflow reactor. All of the runs were carried out at a temperature of about 750° F., a liquid hourly space velocity of about 2.0, and a partial pressure of hydrogen of about 1000 p. s. i. g. The effluent was collected in a pressurized receiver and the naphtha condensed therein. Periodically, the liquid contents of the pressurized receiver were removed (after samples of 100 to 250 cc. had accumulated) and the sulfur content of the desulfurized naphtha samples was determined. This provided a continuous indication of the desulfurization ability of the catalyst as the run progressed and thus indicated catalyst life. The effectiveness of the various catalytic masses prepared by calcination at various temperatures are shown in Table I which follows:

Table I

| Run No. | Catalyst Calcination Temp. | Vol. oil/Vol. cat. | Percent Desulfurization |
|---------|----------------------------|--------------------|-------------------------|
| 1       | 1,850° F.                  | 5.4                | 97                      |
|         |                            | 10.9               | 99                      |
|         |                            | 16.4               | 99                      |
|         |                            | 21.9               | 99                      |
|         |                            | 27.4               | 98                      |
|         |                            | 32.9               | 99                      |
|         |                            | 6.7                | 82                      |
| 2       | not calcined               | 13.6               | 78                      |
|         |                            | 20.5               | 69                      |
|         |                            | 27.4               | 65                      |
|         |                            | 34.3               | 64                      |
|         |                            | 41.2               | 63                      |
|         |                            | 8.3                | 86                      |
|         |                            | 16.6               | 66                      |
| 3       | 1,200° F.                  | 24.9               | 57                      |
|         |                            | 33.2               | 56                      |
|         |                            | 41.5               | 54                      |
|         |                            | 49.8               | 49                      |
|         |                            | 1.7                | 91                      |
|         |                            | 4.0                | 92                      |
|         |                            | 1.8                | 92                      |
| 4       | 1,425° F.                  | 4.2                | 94                      |
| 5       | 1,425° F. <sup>1</sup>     |                    |                         |

<sup>1</sup> Catalyst prepared by calcining mixture containing Ni:Fe molar ratio of 1:1.

The percentage desulfurization of the oil which was obtained with the various catalysts tested is graphically shown in the figure. In this figure the extent of desulfurization is plotted versus the volumes of oil per volume of catalyst. The runs 1, 2, 3, and 4 correspond with catalysts A, B, C, and D, respectively. It is apparent from the graphical presentation in the figure that the intimate mixture of the nickel and iron compounds must be calcined at a temperature of at least 1400° F. to obtain a highly active desulfurization catalyst. X-ray analyses of the catalyst used in runs 1-5 substantiate that a calcination temperature of at least 1400° F. is necessary in order to produce a substantial amount of nickelous ferrite. Run 5 indicates that a highly active nickelous ferrite desulfurization catalyst can be prepared from an intimate mixture of the nickel and iron compounds containing a molar ratio of nickel to iron of 1:1.

A comparison of the nickelous ferrite catalyst with a commercial  $\text{CoO}_3\text{--MoO}_3\text{--Al}_2\text{O}_3$  catalyst was made.

The commercial catalyst, which contained 3%  $\text{CoO}$  and 9%  $\text{MoO}_3$ , was used to hydrodesulfurize a coke still naphtha having a sulfur content of 0.55% and a bromine number of 70 employing the same hydrodesulfurization conditions as used in runs 1-5 i. e. a temperature of 750° F., a space velocity of 2.0, a partial pressure of hydrogen of 1000 p. s. i. g. at a rate of 2000 s. c. f.  $\text{H}_2/\text{bbl}$ . of naphtha. Samples of the desulfurized oil were periodically collected and analyzed for sulfur content and bromine number. The percentage of reduction in the bromine number is hereinafter termed percentage paraffinization. An indication of the selectivity of the catalyst and desulfurization in preference to hydrogenation of the olefins is obtained by dividing the percent desulfurization by the percent paraffinization; when the selectivity is 1.0, the catalyst displays no selectivity whatsoever. In Table II which follows, a comparison between the nickelous ferrite catalyst of run 1 and the commercial catalyst is made.

Table II

| Run No. | Catalyst                         | Vol. oil/Vol. cat. | Percent Desulfurization | Percent Paraffinization | Selectivity <sup>1</sup> |
|---------|----------------------------------|--------------------|-------------------------|-------------------------|--------------------------|
| 1       | Nickelous ferrite                | 5.4                | 97                      | 65                      | 1.5                      |
|         |                                  | 10.9               | 99                      | 80                      | 1.5                      |
| 6       | commercial catalyst <sup>2</sup> | 32.9               | 99                      | 94                      | 1.0                      |
|         |                                  | 6.5                | 97                      | 94                      | 1.0                      |
|         |                                  | 11.9               | 98                      | 94                      | 1.0                      |

<sup>1</sup> Selectivity = Percent Desulfurization ÷ Percent Paraffinization.

<sup>2</sup> Cobalt oxide-molybdenum oxide-alumina.

It is apparent from the above data that nickelous ferrite is an extremely active desulfurization catalyst. The extent of its superiority would be even more pronounced if the desulfurization runs had been carried out at less severe conditions wherein a lesser extent of desulfurization would be obtained. It will further be noted that the nickelous ferrite catalyst is 50% more selective for desulfurization in preference to paraffinization, and therefore the desulfurized gasoline would retain a larger amount of the higher octane number olefins.

The effectiveness of cobaltous ferrite in the hydrodesulfurization of hydrocarbon oils was demonstrated in a number of experiments. These experiments show the extreme importance of using the chemical compound cobaltous ferrite rather than a mere physical mixture of cobalt and iron oxide. Three different catalytic materials were prepared and their effectiveness evaluated for desulfurization and hydrogenation of the olefins present in the olefinic naphtha. Catalyst E was prepared by heating an intimate mixture of  $\text{Co}(\text{NO}_3)_2 \cdot 6\text{H}_2\text{O}$  and



the mixture having a molar ratio of cobalt to iron of 1:2, to a temperature of 1400° F. and maintaining it at that temperature overnight (about 18 hours). The product was identified by X-ray diffraction analysis as consisting of cobaltous ferrite with some ferric oxide. Catalyst G was made in the same manner as catalyst E except that the intimate mixture of cobalt nitrate and ferric nitrate was heated to only 750° F. X-ray diffraction analysis of catalyst G revealed that it contained no cobaltous ferrite. Catalyst F was made in the same manner as catalyst E except that  $\text{CoCO}_3$  and  $\text{Fe}_2\text{O}_3$  were used in place of the nitrates of cobalt and iron. X-ray analysis of catalyst G showed that cobaltous ferrite had been formed.

The catalysts evaluated were prepared by pulverizing the fragments obtained from the heating steps in the preparation of catalysts E, F, and G, and then pelleting the powder to form  $\frac{1}{8}$  inch pellets using about 2% Sterotex. The Sterotex was burned from the pellets at about 850° with air. Catalyst compositions E, F, and G were then evaluated individually. Samples of these cat-

alyst compositions were used to desulfurize a coke still naphtha having a sulfur content of 0.95% and a bromine number of 75 in the apparatus and under the operating conditions previously described. The results obtained with these catalyst compositions are shown in Table III which follows:

Table III

| Run No. | Catalyst       | Percent Desulfurization | Percent Paraffination | Selectivity <sup>a</sup> |
|---------|----------------|-------------------------|-----------------------|--------------------------|
| 7       | E <sup>1</sup> | 91                      | 47                    | 1.9                      |
| 8       | F <sup>1</sup> | 91                      | 41                    | 2.2                      |
| 9       | G <sup>2</sup> | 22                      | 20                    | 1.1                      |

<sup>1</sup> Catalyst had cobaltous ferrite as active component.

<sup>2</sup> Catalyst composition had no cobaltous ferrite, only  $Co_3O_4 + Fe_2O_3$  as a physical mixture.

<sup>a</sup> Selectivity = percent desulfurization ÷ percent paraffination.

The above table shows the excellent ability of cobaltous ferrite for catalyzing the hydrodesulfurization of a hydrocarbon oil. Comparison of the desulfurization results obtained in runs 7 and 8 with run 9 shows the extreme importance of using the chemical compound cobaltous ferrite rather than a physical mixture of cobalt oxide and iron oxide for desulfurizing the oil. A comparison of these same runs further illustrates that low temperatures such as 750° F. cannot be used in preparing cobaltous ferrite and likewise will not produce a composition which is effective as a desulfurization catalyst. The percentage of paraffination of the coke still naphtha should also be noted. When using the cobaltous ferrite catalyst of runs 7 and 8 a selectivity of approximately 2 or higher was obtained, but when using the physical mixture of cobalt oxide and iron oxide as the catalyst the selectivity was only about 1.1. It is important to note, however, that with the cobaltous ferrite catalyst a very high degree of desulfurization can be obtained while minimizing the degree of paraffination of the olefins. This peculiar ability of the cobaltous ferrite catalyst enables a petroleum refiner to desulfurize an olefinic naphtha fraction while minimizing the paraffination of olefins and thus minimizing the loss in octane number of the desulfurized naphtha. The economic advantage of using such a catalyst is obvious.

Thus having described our invention what is claimed is:

1. The method of desulfurizing a hydrocarbon oil containing organic sulfur compounds which comprises contacting said oil in the presence of hydrogen at a temperature between about 600° and 1000° F. with a catalyst containing as the essential component at least one metal ferrite selected from the group consisting of cobaltous ferrite and nickelous ferrite which metal ferrite is prepared by calcining an intimate mixture of a com-

ound affording an oxide of iron and a compound affording an oxide of a metal selected from the class consisting of cobalt and nickel, the intimate mixture containing the metals in the following ratio:

- 5 Molar ratio of cobalt:iron of 0.2 to 2.0:1  
Molar ratio of nickel:iron of 0.2 to 2.0:1

and the metal ferrite being formed by heating the mixture at a temperature between about 1400° to 2000° F. for a period of about 1 to 24 hours.

2. The method of claim 1 wherein said intimate mixture is calcined at a temperature of at least 1800° F.

3. The method of claim 1 wherein the intimate mixture which is calcined contains a molar ratio of cobalt and/or nickel:iron of 0.5:1.

4. The method of claim 1 wherein said metal ferrite is extended upon a carrier.

5. The method of claim 1 wherein said hydrocarbon oil is a petroleum naphtha.

- 20 6. The method of claim 5 wherein said naphtha is an olefinic naphtha.

7. The method of desulfurizing a petroleum naphtha which comprises contacting said naphtha at a temperature between about 600° and 1000° F. and at a pressure of about 100 to 3000 p. s. i. g. in the presence of hydrogen with a catalyst containing as the essential component at least one metal ferrite selected from the group consisting of cobaltous ferrite and nickelous ferrite which metal ferrite is prepared by calcining an intimate mixture of a compound affording an oxide of iron and a compound affording an oxide of a metal selected from the class consisting of cobalt and nickel, the intimate mixture containing the metals in the following ratio:

- 35 Molar ratio of cobalt:iron of 0.5:1  
Molar ratio of nickel:iron of 0.5:1

and the metal ferrite being formed by heating the mixture at a temperature between 1800° and 2000° F. for a period of about 1 to 24 hours.

- 40 8. The method of claim 7 wherein the intimate mixture being calcined is a mixture of nickel oxide and iron oxide.

#### References Cited in the file of this patent

#### UNITED STATES PATENTS

- 45 1,932,174 Gaus et al. Oct. 24, 1933  
1,932,186 Pier et al. Oct. 24, 1933  
1,996,008 Kaehler et al. Mar. 26, 1935

#### FOREIGN PATENTS

- 50 717,301 France Oct. 19, 1931